

Feb. 14, 1939.

D. K. PATTILLOCH

2,147,213

PAPER MAKING PROCESS

Filed May 27, 1937



Inventor:  
Donald K. Pattilloch  
By: Amos, Thies, Olsen & Mecklenburger.

## UNITED STATES PATENT OFFICE

2,147,213

## PAPER-MAKING PROCESS

Donald K. Pattilloch, Neenah, Wis., assignor to  
 Pattilloch Processes, Inc., Boston, Mass., a corporation of Massachusetts

Application May 27, 1937, Serial No. 144,975

11 Claims. (Cl. 92—21)

The present invention relates to an improvement in a process for incorporating starch with paper during its formation, for the purpose of enhancing the strength of the paper, to improve its formation, and to endow it with superior qualities as compared with paper made from the same grade of fiber but in the absence of the starch.

One of the major objects of the present invention is to co-ordinate the addition of the starch and the starch-precipitating chemicals so as to obtain the maximum benefits from the starch addition and particularly to avoid those difficulties which have hitherto stood in the way of successful incorporation of starch with paper fibers during the formation of a paper web on a paper-making machine.

A further object of the invention is to time the addition of the starch and the starch-precipitating chemicals so as to secure the maximum benefits from the starch addition while avoiding those inconveniences and difficulties which arise in the course of the operation of a paper-making machine by reason of the great many variables which are encountered during the operation thereof, such for example as the variables introduced into the operation by the dilution at the mixing box of a paper plant where white water, fresh water, or a mixture of the two in varying proportions is mixed with the concentrated stock derived from the beater.

A further object of the invention is to insure the retention of starch in the forming paper web, which involves beating gelatinized starch with paper fibers in a beater to form a starch-containing furnish, subsequently diluting this furnish to the point of maximum dilution at which it is ready to pass to the wire of the paper-making machine and at the point of maximum dilution, and while the stream is freely flowing, adding thereto, in the order named, aluminum sulfate, and an alkaline material from the group consisting of sodium aluminate, sodium metasilicate and sodium sesquisilicate, or their equivalents, as for example the corresponding potassium salts.

A still further object of the invention is to coordinate the above mentioned operations so as to insure the presence in the diluted furnish at all times of the proper amount of potential aluminum hydroxide or aluminous silicate forming reagents, properly proportioned to the amount of starch present in the diluted furnish to insure the precipitation and bonding to the fibers of the starch which was added in the beater.

Still another object of the invention is to control the above mentioned operations so that a fairly constant hydrogen-ion concentration will be maintained in the diluted furnish which passes to the wire of the paper-making machine, the alkaline material from the group consisting of sodium aluminate, sodium metasilicate, and sodium sesquisilicate, being added at a constant rate which is proportional to the rate of paper production on the wire and which rate is related to the amount of starch present in the furnish and the operating conditions, nature of stock, etc., the aluminum sulfate being added at a varying rate in accordance with the hydrogen-ion concentration of the furnish actually flowing to the head box of the paper-making machine, so that there will always be present in the diluted furnish the correct amount of aluminous-precipitate-forming reagents to precipitate the starch in the furnish and to bond the same to the paper fibers, thereby retaining the starch in the finished sheet.

Other objects of the invention will become apparent from the further description hereinbelow and the hereunto appended claims.

It has already been proposed, by myself as well as others, to introduce starch into paper during its formation. In some of these prior art processes dry starch has been fed into the flowing stream of paper furnish just prior to the admission of the furnish to the head box of the paper machine while also controlling the hydrogen-ion concentration of the flowing stream. It will be noticed, however, that in such a prior art process as for example that disclosed and claimed in my prior Patent No. 1,907,440, of May 9, 1933, the starch was the final ingredient added, and this starch was in the raw condition. It has been found, however, that the retention of starch when thus fed raw is quite insufficient and that considerable quantities of starch are lost in the white water which passes through the wire of the machine and that, even though white water return is used, the retention of the starch is insufficient, particularly because it is not properly bonded to the paper fibers. In another one of my previous patents, No. 2,036,882, of April 7, 1936, I have described a process in which gelatinized starch and aluminum sulfate are added to a beater containing paper-making fibers and beaten therein to form a fiber furnish, this furnish, after discharge from the beater, having sodium aluminate or sodium metasilicate added thereto in order to precipitate aluminum hydroxide or an aluminous silica compound, which carries down the starch and causes its adherence

to the fibers. This last mentioned process has proved successful because it so co-ordinates the order of addition of these materials—namely, the starch and the precipitating agents—as to insure the bonding of the starch to the fiber. It has been found, however, in many paper mills where this process has gone into use, that the rate of dilution of the stock at the mixing box varies from time to time during the operation of the machine, particularly as to the proportions and chemical condition of white water and fresh water used for diluting the stock or furnish, such as its solids-content, colloidalinity and the like. Furthermore, when simultaneously sizing the fibers in the beater by means of the well known method of adding a rosin soap or size and precipitating the same with alum or aluminum sulfate, additional aluminum sulfate is employed to react with the subsequently added sodium aluminate, but the excess aluminum sulfate in the beater is subject to considerable, practically uncontrollable variations. This is caused by the fact that the aluminum sulfate requirements of the size will vary from batch to batch, and in the making up in a commercial beater there will be unavoidable variations in the actual amount of paper fibers present, due to variations in the weight of pulp bales. Furthermore, the excess alum has a distinct tendency to react with the fibers and to become adsorbed thereon, so that it will not be present in properly ionized condition in solution in the water phase of the furnish. In commercially carrying out my prior process of Patent No. 2,036,882, the control was so operated as to maintain a constant hydrogen-ion concentration equivalent to about pH 5.5 to pH 5.7 at the head box of the machine. In order to accomplish this, the sodium aluminate had been added in a varying stream of a solution of constant strength, say 10%, the stream being directed into the dilute stream of furnish flowing between the mixing box and the head box of the machine. However, inasmuch as the addition of the sodium aluminate decreases the hydrogen-ion concentration (hence raises the pH), it was also found that there would be insufficient starch retention and that the increased Mullen strength of the paper would not be apparent. On careful investigation it was discovered that the reason for this was that sufficient alum had been bonded by the fibers, used up by the size, or rendered inert by constituents of the water, so that there would be an insufficient amount of properly ionized aluminum sulfate in the furnish at the time the sodium aluminate was added. I found, as a result of careful tests, that a really successful bonding of starch to the paper fibers can be accomplished only if the starch is precipitated by the correct and proper amount of aluminum hydroxide or aluminum-silica complex, this precipitation taking place at a carefully controlled hydrogen-ion concentration.

I have therefore conceived and developed a marked improvement in a process generally laid down in my prior Patent No. 2,036,882, in that I have modified the procedure in the following respects: Instead of adding the alum to the beater, as I have hitherto done, I now do one of two things; I either add a part of the alum to the beater and the rest of it to the flowing stream of furnish at its point of ultimate dilution or add it all to the diluted furnish, and only then, after I am sure that the right amount of properly ionized aluminum sulfate is present in the diluted furnish, do I add the sodium aluminate or other precipi-

tant. To accomplish this I add the starch to the beater, the starch being in the gelatinized condition, which may be accomplished by boiling or by chemical means, or it may be a modified starch capable of gelling in water, thus producing a starch-containing furnish. This I pass through the Jordan and then to the mixing box of the paper-making machine, where the stock which had been at a concentration of about 4% in the beater is diluted with white water and/or fresh water to a consistency of about  $\frac{1}{2}\%$ . The stock is then allowed to flow through an open launder or pipe to the screens and head box of the paper-making machine. Into this flowing stream of starch-containing furnish I feed, by means of an automatic electrically controlled feeding device, a constant volume of a, say, 10% solution of sodium aluminate or equivalent precipitant, the rate of addition of this solution being in proportion to the rate at which paper is being made. A few feet ahead of the point of addition of, for example, the sodium aluminate I add a solution, of say 10%, of aluminum sulfate, in the form known in this art as "paper-maker's alum", the addition of which solution however is varied in accordance with the hydrogen-ion concentration as measured at the head box of the machine. How this control is accomplished will be described in greater detail in connection with the hereunto annexed drawing, which is, respectively:

Fig. 1, a diagrammatic flow sheet of my present improved process; and

Fig. 2, a similar flow sheet illustrating my prior process of Patent No. 2,036,882, so that the difference between the two processes can be most accurately and easily made apparent.

Describing my present invention in connection with Fig. 1, it will be seen that I have provided a beater 3, having thereon indicated that the consistency of the fibers is at about 4%. Into this beater there is fed an appropriate amount of starch 4 and, if desired, sufficient alum 5 to take care of the precipitation of size which might have been used. I prefer however to add only a slight excess of alum at this point. Where I mention alum, it is of course to be understood that I mean the so-called paper maker's alum. The beater furnish at about 4% consistency and containing an amount of starch which for example very advantageously can be equal to 4% of the dry weight of the fibers, but which may vary from 2% up to about 10%, depending upon the results desired, is, after proper beating, sent through the Jordan 6 and thence directed to the mixing box 7, at which point it is diluted by means of white water, fresh water, or a mixture of the two, coming from the white-water collecting sump 8, being pumped to the mixing box 7 by means of the pump 9 through the pipe 10. The fresh-water supply has been diagrammatically illustrated as being a tank 11, although of course it will be obvious that this is merely the regular source of water supply of the mill. In the mixing box 7 the furnish is diluted to a consistency of about  $\frac{1}{2}\%$  and in that condition will flow through the launder or pipe 12 toward the head box 13. There is provided a tank 14 of, say, 10% alum solution, this solution being fed through the pipe 15 and the automatic control valve 16 into the launder 12, as indicated in the drawing. The valve 16 is under the control of a hydrogen-ion control device which is a standard piece of equipment consisting of an electrical instrument and a suitable thermionic tube amplifier and is diagrammatically indicated at 17, the electrode 18 of the

instrument being immersed in the head box 13. The valve 16 therefore will open and close in accordance with the alum requirements of the operation. A little further down along the launder or pipe on its way to the head box, say at a distance of from 3 to 10 feet, there is the point of introduction of the sodium aluminate, or other precipitant, which flows from the storage tank 19 through the pipe 20 and through the flow-control meter 21. This flow-control meter is connected through the electrical control 22 with the operating mechanism which controls the speed of the wire 23. The precipitant solution is at about 10% concentration and is fed at such a rate that if, for example, the rate of paper production is 1600 pounds of dry paper per hour, it will feed approximately 20 pounds per hour of sodium aluminate, or appropriate amounts of other precipitant, into the diluted furnish. This will suffice to throw down or precipitate approximately 64 pounds of starch, which is 4% on the weight of the dry paper being made. In other words, the optimum ratio of starch to sodium aluminate is about 3.5 to 1; to sodium metasilicate it is about 2.5 to 1, and to sodium sesquisilicate about 3 to 1. The paper, after leaving the wire, is of course picked up by the usual couch roll and then passed through the presses and driers 24 and finally reeled up on a reel 25.

30 The range of starch to paper may be from 2% to 10%, but it has been found that the addition of about 4% of starch yields the greatest practical return for the money expended. In other words, the benefits obtained with that percentage of starch are at their best. The amount of sodium aluminate may be from 1% to 1½%, or substantially in the ratio above set forth, the percentage of other precipitants mentioned being in proportion.

40 The particular advantage in operating as just described is that there will always be insured the precipitation of the right amount of aluminous compound, such as hydroxide or complex silicate, hereinafter referred to as aluminum-silicon complex, to produce the best precipitating effect upon the starch.

Having now described my invention in connection with sodium aluminate, I wish it to be thoroughly understood that I may also operate in a similar manner by using a solution of sodium metasilicate or sodium sesquisilicate instead of the sodium aluminate. The hydrogen-ion control when using sodium aluminate should show a pH of from about 5.5 to 6 in the head box of the machine, while with sodium metasilicate or sesquisilicate it is better to work out a pH of about 6.8, but at any rate the furnish should not be allowed to become alkaline, as this might deleteriously affect the size which might have been added in the beater. By size I mean, of course the usual sodium compound of rosin as precipitated by aluminum sulfate in an insoluble form on the fiber.

In order to exemplify the difference between my present process and that which I have described in my previous Patent No. 2,036,882, I shall just briefly review this patent in connection with Fig. 2 of the present specification, corresponding figures being used, properly primed to distinguish from my present invention. Where the numbers are not primed, the arrangement and devices are the same. Referring to Fig. 2, therefore, I provide a beater 3 in which the fibers are at a consistency of about 4%, adding gelatinized starch 4, so that there will be about 4%

of starch on the dry weight of the fibers in the beater. I also incorporate alum 5 in the beater, but there is no other point of addition of alum in this prior process. In other words, I put all the alum which I intend to use right into the beater and beat it with the starch and the fibers. The mixture in the beater, which then consists of fibers, gelatinized starch and alum (and also any size with which the fibers may have been treated), is fed through the Jordan 6 into the mixing box 7 of the machine, where it is diluted with water flowing through the pipe 10 under the influence of pump 9, this water being either fresh water, white water, or a mixture thereof, exactly as in the case of Fig. 1. The diluted stock, at a consistency of about ½%, flows through the launder or pipe 12 and receives an addition of precipitant from the tank 19, this solution flowing through the line 20 and the valve 21, which in this case is under the control of the electrical control device 17' which has its electrode 18 in the head box 13 of the machine. The precipitant thus reacts with the alum already present in the diluted furnish to precipitate the alum, forming an aluminous precipitate. By reason of the white water returned and the great variation in the amount of fresh water with which the latter is diluted, the condition of the stock varies from time to time as it flows through the launder or pipe 12. If everything is working properly, of course, my prior process gives excellent results, and the Mullen strength of the paper, which ordinarily may be only about 26, will be raised to as high as 42 to 43, based upon a 20-pound bond paper. However, when operating in accordance with my prior process just described, it has often happened that, although the pH was properly controlled at about 5.7 and the precipitant was added strictly in accordance with the reading of the control instrument 17' and the setting of the valve 21', the Mullen test would suddenly drop to as low as 35 for no apparent reason. I have now found that the reason for this was that, due to the variation in white water return and also due to variables in the making up of the beater furnish, there would be an insufficient amount of properly ionized aluminum sulfate in the ½% diluted stock in the launder or pipe 12 to react with the precipitant. Obviously, if there is not enough aluminum sulfate, the precipitant will raise the pH of the solution in the head box, and hence the electrical control will throttle down the amount of precipitant fed, as otherwise, because of its alkalinity, the pH would continue to rise. Naturally, if there were insufficient aluminum sulfate, there would also be insufficient precipitant, so that there would be a precipitation of the aluminous compounds of only diminished amount, which would be insufficient properly to precipitate the starch.

This condition I have now completely remedied by practicing the invention which I have disclosed herein in connection with Fig. 1, where I insure the presence of the proper amount of alum by feeding the sodium aluminate or other herein named precipitating reagent at a constant rate directly proportioned to the production rate of the machine, but feed alum ahead of the precipitant into the flowing stream of diluted stock under the control of the control instrument 17 and valve 16. In this way I can maintain the Mullen strength at about 42 for 20-pound stock without any difficulty whatever.

To explain the variations in beater furnishes,

it should be remembered that when making up a beater furnish the sulphite and other stocks used are measured in terms of bales, laps, etc. rather than weighed, and these bales, etc. vary considerably in weight, so that it will not always be possible to maintain an exact predetermined consistency in the beaters. For example, a so-called "2000-pound" beater furnish may vary, so far as fibers are concerned, between 1900 and 2200 pounds because of these variations. The sizing and other chemicals, however, are weighed, and hence usually are present in the predetermined quantities. The ratio of these chemicals to the fiber will thus vary considerably, and there are thus introduced into the operation a number of unpredictable variables. Furthermore, size varies from time to time, and hence the alum requirements for precipitation likewise vary. Further variables are introduced into the operation by the nature of the water employed, for diluting the stock after its removal from the beater, i. e., in the mixing box 1. Obviously if all white water is used and this has, for instance, a pH of 5.8, there will be one effect, and if all fresh water is used and this has a pH, say, of 7.2, there will be another effect, with a further variation caused when mixtures of fresh and white water are employed. The white water contains colloidal matter, while the fresh water is usually fairly free from such material but also differs from the white water, and on different days, in total solids content, hardness, etc.

By operating as hereinabove described, however, I can overcome these variations, which from a commercial point of view is of paramount importance and constitutes what I believe to be the greatest single advance in this particular field that has been made to date.

There is also another very important advantage in operating as I have herein described, and that lies in the fact that I not only can increase the Mullen strength of the paper but also its tearing strength, folding endurance, and tensile strength. The reason for this is that, by precipitating the starch onto the fibers, I obtain an effect which is quite analogous to the hydration of the fibers; that is to say, the stock becomes less free, which gives a better formation and a stronger sheet, as is well known. Formerly, and without the use of my invention, it was necessary to beat the fibers for a much longer time and to subject them to more severe jordaning in order to hydrate them. In so doing, while they would increase in diameter due to their having imbibed sufficient water to effect the hydration or gelatinization, they were, at the same time, reduced in length, and it is the length of fibers that controls the tear, fold and tensile strength, while the hydration effect controls the Mullen strength and to some extent the wet tensile strength. By my present process, however, I can beat the fibers for a much shorter length of time and subject them to a less vigorous Jordan treatment, because I do not have to depend upon beating and jordaning for the hydration and gelatinization effect, and by thus reducing the mechanical preparation of the fiber I get a far better fiber length, which naturally improves the above mentioned qualities of the paper.

Just as an example of how greatly the present invention is capable of increasing the wet tensile strength of the paper product, it may be mentioned that in a recently developed wet strength test, the wet strength was increased about 2000%. This test is made by obturating

the bottom of an open 3-inch cylinder about 24 inches high with a disk of the paper to be tested and then filling the cylinder to a predetermined height with water at 70° F., not less than 3.0 kilograms of water being used, so that the paper is thus subjected to a dead weight of this amount of water over the entire area of the 3-inch disk. The time when the paper breaks under this load is measured in minutes and seconds. A given grade of butcher's wrapping paper made by customary methods had a test of 9 minutes, but when the same stock was made into paper with the use of the present invention it required 190 minutes, or an increase of 181 minutes, equal to 2000%.

In order to complete the disclosure, I am here mentioning the approximate chemical formulas of the precipitants employed by me. Thus the sodium aluminate is a commercially obtainable product and has the formula  $Na_2Al_2O_4$ . The available commercial grade usually gives the following approximate chemical analysis:

|                                       | Per cent |
|---------------------------------------|----------|
| Soluble silica, $SiO_2$ -----         | 0.50     |
| Sodium hydroxide, $NaOH$ excess-----  | 7.99     |
| Sodium carbonate, $Na_2CO_3$ -----    | 1.04     |
| Sodium aluminate, $Na_2Al_2O_4$ ----- | 87.13    |
| Insoluble -----                       | 1.42     |
| Sodium potassium tartrate-----        | 1.92     |
|                                       | 30       |
|                                       | 100.00   |

The sodium metasilicate and sesquisilicate are also commercial products. Sodium metasilicate is a definite chemical compound having the formula  $Na_2SiO_3 \cdot 5H_2O$ . It has been described together with a number of its other hydrates in United States Patent No. 1,898,707. Sodium sesquisilicate has a molecular formula of



and contains about 36.89%  $Na_2O$ , 23.83%  $SiO_2$ , and 39.27% water. It is described in United States Patent No. 1,948,730. An alternative formula is  $Na_3HSiO_4 \cdot 5H_2O$ . Obviously, I can use more than one of these materials, i. e., the aluminate and the silicate, at the same time, introducing them separately, or together, or each under its own control.

Summing up my invention, therefore, it not only assures a better grade of paper with the same amount of fiber and a paper which is of improved physical properties, such as Mullen bursting strength, tear strength, folding endurance and tensile strength, but which also has a closer and better formation and smoother surface, and which is far superior in every respect. The essential point to be remembered is that I have now solved the difficulties which have hitherto accompanied the carrying out of my prior inventions, in that I have successfully overcome the many variables which are encountered in the commercial operation of a paper machine, and for this invention I claim:

1. The improvement in incorporating starch in paper during its formation which comprises the steps of mixing gelatinized starch with paper fibers to form a starch-containing furnish, diluting the furnish to substantially paper-forming consistency, adding aluminum sulfate thereto while the furnish is flowing in a stream, and then similarly adding a sufficient amount of a precipitant from the group consisting of sodium aluminate, sodium metasilicate and sodium sesquisilicate thereto to form an aluminous precipitate by

the substantially complete reaction of both added ingredients in the furnish but keeping the furnish on the acid side of neutrality, whereby the starch is precipitated upon the fibers, and forming a paper web therefrom.

2. The improvement in incorporating starch in paper during its formation which comprises the steps of mixing gelatinized starch with paper fibers to form a furnish containing fibers at about 4% consistency, diluting this furnish after removal from the beater to a consistency of about  $\frac{1}{2}\%$ , flowing the diluted furnish toward the wire of a paper-making machine and while thus flowing adding, successively, aluminum sulfate and a precipitant from the group consisting of sodium aluminate, sodium metasilicate and sodium sesquisilicate thereto in substantially stoichiometrically balanced amounts to form thereon an aluminous precipitate by the reaction of both added ingredients but keeping the furnish on the acid side of neutrality, whereby the starch is precipitated onto the fibers, and forming a paper web therefrom.

3. The improvement in incorporating starch in paper during its formation which comprises the steps of mixing, in a beater, cellulosic fibers, water and starch to form a paper furnish containing fibers and gelatinized starch, transferring this furnish continuously to a point of dilution and then diluting it to a consistency suitable for web formation, flowing the diluted furnish toward the wire of a paper-making machine and while thus flowing introducing thereinto a precipitant from the group consisting of sodium aluminate, sodium metasilicate, and sodium sesquisilicate, at a constant rate predetermined by the rate of paper production of the machine, measuring the hydrogen-ion concentration of the furnish as it enters the head box of the machine and adding a solution of aluminum sulfate to the flowing furnish at a point ahead of that of the introduction of the precipitant in an amount sufficient to react therewith so as to maintain the predetermined hydrogen-ion concentration at the head box, whereby a sufficient amount of aluminous precipitate will be formed in the furnish properly to bond the starch to the fibers, the hydrogen-ion concentration hereinabove mentioned being that corresponding to a pH of from about 5.5 to 6.8.

4. The improvement in incorporating starch in paper during its formation which comprises the steps of beating paper-making fibers in a beater with from about 2% to 10% of gelatinized starch based on the dry weight of the fibers, subsequently diluting the resultant starch-containing furnish to substantially its ultimate consistency, and then adding separately thereto stoichiometrically balanced amounts of aluminum sulfate and a precipitant from the group consisting of sodium aluminate, sodium metasilicate and sodium sesquisilicate to precipitate the starch, while keeping the furnish thereby at a pH of from about 5.5 to 6.8.

5. The improvement in incorporating starch in paper during its formation which comprises the steps of beating paper-making fibers in a beater with the addition of from about 2% to 10% of gelatinized starch based on the dry weight of the fiber, diluting the thus produced starch-containing furnish to a consistency suitable for paper-web formation, and prior to its introduction into the head box of the paper-making machine adding aluminum sulfate and sodium aluminate thereto in stoichiometrically balanced amounts to precipitate sufficient aluminum hydrate to bond the starch to the fibers, while maintaining

a predetermined hydrogen-ion concentration of from about pH 5.5 to 6.8 at the head box of the machine.

6. The improvement in incorporating starch in paper during its formation which comprises the steps of beating paper-making fibers in a beater with the addition of from about 2% to 10% of gelatinized starch based on the dry weight of the fiber, diluting the thus produced starch-containing furnish to a consistency suitable for paper-web formation, and prior to its introduction into the head box of the paper-making machine adding aluminum sulfate and sodium metasilicate thereto in stoichiometrically balanced amounts to precipitate sufficient aluminous precipitate to bond the starch to the fibers, while maintaining a predetermined hydrogen-ion concentration of from about pH 5.5 to 6.8 at the head box of the machine.

7. The improvement in incorporating starch in paper during its formation which comprises the steps of beating paper-making fibers in a beater with the addition of from about 2% to 10% of gelatinized starch based on the dry weight of the fiber, diluting the thus produced starch-containing furnish to a consistency suitable for paper-web formation, and prior to its introduction into the head box of the paper-making machine adding aluminum sulfate and sodium sesquisilicate thereto in stoichiometrically balanced amounts to precipitate sufficient aluminous precipitate to bond the starch to the fibers, while maintaining a hydrogen-ion concentration of from pH 5.5 to about pH 6.8 at the head box of the machine.

8. The process of making paper containing starch which comprises the steps of beating paper-making fibers and gelatinized starch in a beater together with aluminum sulfate to produce a starch-containing fiber furnish, diluting the same to its final consistency suitable for web formation and adding thereto an amount of a precipitant from the group consisting of sodium aluminate, sodium metasilicate and sodium sesquisilicate, based on the rate of paper production, while augmenting the aluminum sulfate content of the diluted furnish just prior to the addition of the precipitant so as to insure the presence in the diluted furnish of sufficient aluminum sulfate to react with all of the precipitant, and to maintain the hydrogen-ion concentration of the furnish on the acid side of neutrality.

9. In the process of making paper containing starch which comprises the steps of beating paper-making fibers and gelatinized starch in a beater with aluminum sulfate to produce a fiber furnish containing X% of starch, and, after removal from the beater, diluting the furnish to the ultimate consistency at which it is to be fed to the wire of a paper-making machine, flowing the diluted furnish toward the wire in a stream and adding thereto Y% of sodium aluminate at a rate adjusted to the speed of paper production per hour, the ratio of X to Y being as about 3.5:1, and also feeding into said stream, ahead of the sodium aluminate, sufficient additional aluminum sulfate to insure the presence of a sufficient amount thereof to react with all of the sodium aluminate, the control of the addition of said aluminum sulfate being based on a maintained hydrogen-ion concentration of pH 5.5 to 6 at the head box of the paper machine.

10. In the process of making paper containing starch which comprises the steps of beating paper-making fibers and gelatinized starch in a beater with aluminum sulfate to produce a fiber

furnish containing  $X\%$  of starch, and, after removal from the beater, diluting the furnish to the ultimate consistency at which it is to be fed to the wire of a paper-making machine, flowing the diluted furnish toward the wire in a stream and adding thereto  $Y\%$  of sodium metasilicate at a rate adjusted to the speed of paper production per hour, the ratio of  $X$  to  $Y$  being as about 2.5:1, and also feeding into said stream, ahead of the sodium metasilicate, sufficient additional aluminum sulfate to insure the presence of a sufficient amount thereof to react with all of the sodium metasilicate, the control of the addition of said aluminum sulfate being based on a maintained hydrogen-ion concentration of about pH 6.8 at the head box of the paper machine.

11. In the process of making paper containing starch which comprises the steps of beating paper-making fibers and gelatinized starch in a

beater with aluminum sulfate to produce a fiber furnish containing  $X\%$  of starch, and, after removal from the beater, diluting the furnish to the ultimate consistency at which it is to be fed to the wire of a paper-making machine, flowing the diluted furnish toward the wire in a stream and adding thereto  $Y\%$  of sodium sesquisilicate at a rate adjusted to the speed of paper production per hour, the ratio of  $X$  to  $Y$  being as about 3:1, and also feeding into said stream, ahead of the sodium sesquisilicate, sufficient additional aluminum sulfate to insure the presence of a sufficient amount thereof to react with all of the sodium sesquisilicate, the control of the addition of said aluminum sulfate being based on a maintained hydrogen-ion concentration of about pH 6.8 at the head box of the paper machine.

DONALD K. PATTILLOCH.